

Dec. 28, 1965

J. J. JESMONT ETAL

3,226,266

METHOD OF MAKING PERMANENT MAGNETS

Filed Feb. 7, 1962

FIG. 1



FIG. 2



INVENTORS  
JOHN J. JESMONT  
SAMUEL WEIMERSHEIMER

BY *Lindsey, Prutzman and Hayes*  
ATTORNEYS

3,226,266  
**METHOD OF MAKING PERMANENT MAGNETS**  
 John J. Jesmont, Spotswood, and Samuel Weimersheimer,  
 Rockaway, N.J., assignors to U.S. Magnet & Alloy  
 Corporation, Bloomfield, N.J., a corporation of  
 Delaware

Filed Feb. 7, 1962, Ser. No. 171,641  
 4 Claims. (Cl. 148—3)

The present invention relates to permanent magnets and more particularly to magnets of ferrous alloys containing aluminum, nickel and cobalt having improved magnetic properties, and to alloys therefor.

Alloys containing 6 to 11 percent by weight aluminum, 12 to 20 percent by weight nickel, 16 to 30 percent by weight cobalt, up to 7 percent by weight copper and the remainder principally iron, generally known as Alnico V, have been widely utilized in the production of permanent magnets. By chill casting of the alloy under controlled conditions, it has been possible to produce substantially unidirectionally grained castings which develop high magnetic properties. One of the principal problems in achieving optimum properties is the tendency for the casting to develop a multi-phase microstructure, whereas the ideal structure magnetically is one consisting entirely of the alpha phase.

Accordingly, the heat treatment of Alnico alloys of the above analysis under closely controlled conditions has been necessary to avoid multi-phase structure and to achieve the desired alpha phase. At temperatures of about 2350° F. and about 1650° F. only the alpha phase exists but prolonged heating at temperatures of about 1525 to 1600° F. produces a beta phase and at temperatures of about 1750 to 2300° F. precipitates the gamma phase. Various elements have been proposed in an effort to minimize the gamma phase problem and improve the magnetic properties including zirconium and silicon.

It is an object of the present invention to provide a novel permanent magnet having greatly enhanced magnetic properties and characterized by substantial freedom from multi-phase structure.

Another object is to provide an alloy and method for making permanent magnets which permits the facile casting of the magnet bodies and which may be readily heat-treated without extensive normalizing treatment at high temperatures to produce magnets of high magnetic strength and free from multi-phase structure.

A further object is to provide an alloy which can be readily cast into a body having a unidirectionally oriented grain structure and heat-treated to provide a magnet having greatly enhanced magnetic properties.

Other objects and advantages will be readily apparent from the following detailed specification and appended claims, and by reference to the attached drawing wherein:

FIG. 1 is a graph showing the demagnetization curves of directionally grained magnets and random-grained magnets of the alloy of the present invention and that of directionally grained magnets of conventional Alnico V alloy not incorporating the additive elements of the present invention; and

FIG. 2 is a representation of the grain structure of directionally grained magnets produced from the alloy of the present invention.

It has now been found that the foregoing and related objects can be attained by incorporation of 0.15 to 0.50 percent by weight columbium and 0.15 to 0.50 percent by weight titanium in an alloy containing 6 to 11 percent by weight aluminum, 12 to 20 percent by weight nickel, 16 to 30 percent by weight cobalt, up to 7 percent by weight copper and the remainder substantially entirely iron with the usual impurities, such as silicon and carbon. The

columbium and titanium are preferably employed in the range of 0.20 to 0.35 percent by weight of each for optimum effect.

The preferred alloys of this invention are those ferrous base alloys containing 8.0 to 8.8 percent by weight aluminum, 13.0 to 14.0 percent by weight nickel, 23.5 to 25.0 percent by weight cobalt, 1.50 to 3.50 percent by weight copper, to which the columbium and titanium are added in the range of 0.15 to 0.50 percent by weight each, and most desirably 0.20 to 0.35 percent by weight.

In the alloys of the present invention, the coercive force and mechanical properties are significantly enhanced while the problems attendant to producing a single-phase microstructure are greatly reduced, thus enabling the facile production of superior permanent magnets. By the present invention, directionally grained magnets having a maximum energy product ( $BH_{max}$ ) of at least 6.0 million gauss-oersteds, and generally at least 7.0 million gauss-oersteds are readily produced. Using preheated chill molds with little transverse heat loss, magnets have been produced in commercial operation having a maximum energy product of 7.5 to 8.5 million gauss-oersteds.

The alloy of the present invention may also be cast to produce random-grained magnets in conventional baked sand molds with resultant properties of coercive force and maximum energy product equivalent to commercial directionally grained Alnico V magnets heretofore available. By the present invention, random-grained magnets having a coercive force of at least 700 oersteds and a maximum energy product of at least  $5.0 \times 10^6$  gauss-oersteds are readily obtained.

FIG. 1 of the attached drawing is a graph showing the demagnetization curves of directionally grained magnets (A) and of random-grained magnets (B) cast in commercial operation from the alloy of the present invention as compared with the demagnetization curve of directionally grained magnets commercially produced from alloys theretofore utilized (C). FIG. 2 is a representation of the grain structure of directionally grained magnet bodies commercially cast from the alloy and evidences but six columnar grains across the transverse section.

The following is a specific example of an alloy of the present invention which has proven highly advantageous for producing superior magnets:

| Element:                              | Percent, by weight |
|---------------------------------------|--------------------|
| Aluminum                              | 8.3                |
| Nickel                                | 13.3               |
| Cobalt                                | 24.5               |
| Copper                                | 2.9                |
| Titanium                              | 0.2                |
| Columbium                             | 0.3                |
| Remainder iron with minor impurities. |                    |

Indicative of the properties of typical magnets produced from the alloy of the present invention are the data set forth in Table One below:

TABLE ONE  
*Magnetic properties of magnets*

| Magnet          | Residual Flux Density, Br, gauss | Coercive Force, Hc Oersteds | Maximum Energy Product BH max, Gauss-Oersteds ( $\times 10^6$ ) |
|-----------------|----------------------------------|-----------------------------|-----------------------------------------------------------------|
| Directionalized | 13,370                           | 744                         | 6.9                                                             |
| Do              | 13,020                           | 860                         | 8.15                                                            |
| Do              | 13,400                           | 810                         | 7.3                                                             |
| Random          | 12,500                           | 730                         | 5.3                                                             |
| Do              | 12,800                           | 750                         | 5.7                                                             |
| Do              | 12,400                           | 720                         | 5.5                                                             |

For casting directionally grained magnet bodies in ac-

cordance with the preferred aspect of the present invention, the alloy preferably is superheated to a temperature of 2850 to 3450° F. and cast in molds which have been preheated to a temperature of 1200 to 2700° F. and the superheat extracted through a chill plate at one end to achieve a unidirectionally grained structure.

The alloy of the present invention is particularly advantageous in that it substantially ameliorates the problems attendant to avoiding the production of a multi-phase micro-structure in the magnets so as to obtain optimum magnetic properties. More particularly, it has been found that the castings of the present invention do not require normalizing treatment at elevated temperatures above about 2300° F. to eliminate any gamma phase precipitation which may have occurred during casting. Furthermore, the castings of the new alloy may be heat-treated at temperatures and times which enable facile and highly effective production of the magnetized bodies due to eliminating major problems in the development of a multi-phase structure during heat-treatment.

In particular, the magnet castings of the new alloy are magnetically stressed by soaking at a temperature of 1650 to 1700° F. for fifteen to twenty minutes and cooling in a magnetic field parallel to the principal grain direction to a temperature of about 1200° F. in about ten to fifteen minutes. Subsequently, the castings are coercively aged or drawn at a temperature of 1100 to 1150° F. for three to ten hours and then at 1025 to 1100° F. for ten to twenty-four hours, after which the castings were cooled to room temperature. The conditions for the magnetic stress treatment are quite critical, but the conditions for the coercive aging are relatively broad and free from any significant problems.

The coercive aging precipitates intermetallic compounds in the matrix and enhances the magnetic properties which have been developed by freezing of the domains during soaking and alignment thereof during cooling in the magnetic field parallel to the direction of grain growth.

Indicative of the efficacy of the present invention are the following specific examples:

#### EXAMPLE ONE

An alloy containing 8.3 percent by weight aluminum, 13.3 percent by weight nickel, 24.5 percent by weight cobalt, 2.9 percent by weight copper, 0.2 percent by weight titanium, 0.3 percent by weight columbium, and the remainder principally iron with carbon and silicon impurities of less than 0.12 percent was superheated to a temperature of about 3350° F. and cast in refractory molds preheated to a temperature of about 2050° F. and using a chill plate to produce speaker plugs 0.759 inch in diameter and 0.522 inch in length. Upon inspection of a transverse section, the castings were found to be unidirectionally grained and to have only six columnar grains.

The castings were then normalized at about 1700° F. for one-half hour and cooled in a magnetic field parallel to the axis of grain orientation for about fifteen minutes. The magnet bodies were then subjected to coercive aging at a temperature of about 1100° F. for about two hours and at about 1025° F. for twenty hours.

The magnets had a residual flux density ( $B_r$ ) of 13,400 gauss, a coercive force ( $H_c$ ) of 810 oersteds and a maximum energy product ( $BH_{max}$ ) of  $8.1 \times 10^6$  gauss-oersteds.

#### EXAMPLE TWO

An alloy containing 8.5 percent by weight aluminum, 13.0 percent by weight nickel, 23.8 percent by weight cobalt, 2.6 percent by weight copper, 0.3 percent by weight titanium, 0.2 percent by weight columbium, and the remainder principally iron was superheated to a temperature of about 3450° F. and cast in refractory molds preheated to a temperature of about 2000° F. and using a chill plate to produce speaker plugs two inches in diameter and two inches in length. Upon inspection of a transverse section, the castings were found to be unidirectionally grained and to have only 40 columnar grains.

The castings were then heat-treated similarly to those in Example One.

The magnets had a residual flux density ( $B_r$ ) of 13,200 gauss, a coercive force ( $H_c$ ) of 810 oersteds, and a maximum energy product ( $BH_{max}$ ) of  $7.60 \times 10^6$  gauss-oersteds.

#### EXAMPLE THREE

The alloy of Example One was cast into speaker plugs of the same size in conventional sand molds according to conventional practice. The resultant castings were then magnetically heat-treated under conditions substantially identical to those in Example One.

The resultant magnets had a residual flux density ( $B_r$ ) of 12,750 gauss, a coercive force ( $H_c$ ) of 690 oersteds and a maximum energy product ( $BH_{max}$ ) of  $5.45 \times 10^6$  gauss-oersteds.

#### EXAMPLE FOUR

An alloy containing 8.3 percent by weight aluminum, 13.6 percent by weight nickel, 24.3 percent by weight cobalt, 2.9 percent by weight copper, 0.15 percent by weight titanium and 0.2 percent by weight columbium was cast in conventional sand molds to form speaker plugs 0.998 inch in diameter and 0.64 inch in length.

The resultant castings were heat-treated substantially in accordance with the conditions in Example One. The resultant magnets were found to have a residual flux density ( $B_r$ ) of 12,500 gauss, a coercive force ( $H_c$ ) of 715 oersteds and a maximum energy product ( $BH_{max}$ ) of  $5.6 \times 10^6$  gauss-oersteds.

As can be seen from the foregoing specific examples and detailed specification, the alloy of the present invention produces magnets having magnetic properties superior to those of conventional Alnico V alloys and may be utilized to cast unidirectionally grained structures having greatly enhanced magnetic properties over prior commercial directionally grained magnets. Additionally, the new alloy does not require as close control over temperatures and times to produce the desired alpha phase microstructure.

We claim:

1. The method of making single-phase unidirectionally columnar grained magnets comprising: introducing into one end of mold chambers opening at the other end on a chill plate a ferrous alloy containing about 6.0 to 11.0 percent by weight aluminum, 12.0 to 20.0 percent by weight nickel, 16.0 to 30.0 percent by weight cobalt, up to 7.0 percent by weight copper, 0.15 to 0.50 percent by weight titanium, 0.15 to 0.50 percent by weight columbium, and the remainder being substantially all iron with minor impurities; chilling said ferrous alloy substantially through said chill plate to form magnet bodies of the desired configuration with unidirectionally columnar grains; magnetically stressing said magnet bodies by soaking at a temperature of about 1650 to 1700° F. for about fifteen to twenty minutes and cooling in a magnetic field parallel to the principal grain direction to a temperature of about 1200° F. in a period of about ten to fifteen minutes; coercive aging said magnet bodies at a temperature of about 1100 to 1150° F. for three to ten hours and thereafter at a temperature of about 1025 to 1100° F. for ten to twenty-four hours to precipitate intermetallic compounds in the matrix; and cooling to room temperature.

2. The method in accordance with claim 1 wherein said copper constitutes about 1.5 to 3.5 percent by weight of said alloy.

3. The method in accordance with claim 1 wherein said ferrous-base alloy contains about 8.0 to 8.8 percent by weight aluminum, 13.0 to 14.0 percent by weight nickel, 23.5 to 25.0 percent by weight cobalt, up to 7.0 percent by weight copper, 0.15 to 0.50 percent by weight titanium, 0.15 to 0.50 percent by weight columbium, and the remainder being substantially all iron with minor impurities.

4. The method in accordance with claim 1 wherein said ferrous-base alloy contains about 8.0 to 8.8 percent

by weight aluminum, 13.0 to 14.0 percent by weight nickel, 23.5 to 25.0 percent by weight cobalt, up to 7.0 percent by weight copper, 0.20 to 0.35 percent by weight titanium, 0.20 to 0.35 percent by weight columbium, and the remainder being substantially all iron with minor impurities.

|           |         |                |       |           |
|-----------|---------|----------------|-------|-----------|
| 2,499,861 | 3/1950  | Hansen         | ----- | 148—102 X |
| 2,499,862 | 3/1950  | Hansen         | ----- | 75—124    |
| 2,694,166 | 11/1954 | Hadfield       | ----- | 148—102 X |
| 2,797,161 | 6/1957  | Ireland et al. | ----- | 75—124    |

## FOREIGN PATENTS

|         |        |         |
|---------|--------|---------|
| 601,597 | 7/1960 | Canada. |
|---------|--------|---------|

## References Cited by the Examiner

## UNITED STATES PATENTS

|           |        |       |       |         |    |
|-----------|--------|-------|-------|---------|----|
| 2,161,926 | 6/1939 | Jonas | ----- | 148—102 | 10 |
| 2,323,944 | 7/1943 | Snoek | ----- | 148—102 |    |

|                                  |
|----------------------------------|
| DAVID L. RECK, Primary Examiner. |
|----------------------------------|

|                                                   |
|---------------------------------------------------|
| MARCUS U. LYONS, ROGER L. CAMPBELL,<br>Examiners. |
|---------------------------------------------------|